# EUROPEAN PATENT SPECIFICATION

(11) **EP 0 825 273 B1**
(45) Date of publication and mention of the grant of the patent: **31.10.2001**
(21) Application number: 97305993.4
(22) Date of filing: 06.08.1997
(51) Int. Cl.: C23C 4/12

(54) **Coating substrates with high temperature ceramics**
Beschichtung von Substraten mit hochtemperaturkeramischen Materialien
Revêtement de substrats avec des céramiques à haute température

(30) Priority: 20.08.1996 GB 9617441
(43) Date of publication of application: 25.02.1998
(73) Proprietor: The BOC Group plc, Windlesham Surrey GU20 6HJ (GB)
(72) Inventor: Creffield, G.K., Chessington, Surrey, KT9 1AY (GB); Cole, M.A., Banstead, Surrey, SM7 3PJ (GB)
(74) Representative: Gough, Peter

(56) References cited:
- EP-A- 0 612 567
- EP-A- 0 621 079
- DE-A- 3 843 436
- GB-A- 1 115 738
- US-A- 4 006 838

## Description

The present invention relates to a method of coating a substrate with high temperature ceramics.

Throughout this specification the expression "high temperature ceramics" is intended to encompass oxides, carbides and nitrides of metals such as chromium, aluminium and zirconium having a melting point above 1800°C.

Chromium oxide has been plasma-sprayed on substrates for many years for applications in such industries as the aerospace and automobile industries.

A further need for relatively thick, high hardness and low porosity chromium oxide coatings is in the print roller industry. In this industry, coatings are usually laser engraved thereby producing indents which are designed to hold ink. The harder and thicker the coating, the greater the density of holes that can be achieved. Atmospheric plasma spraying has produced coating densities between 90- 95% theoretical values, but this allows aggressive gases to penetrate the open porosity and damage both the coating and substrate material. Considerable work has been attempted to reach gas tightness in plasma-sprayed chromium oxide coatings using vacuum plasma spraying, post heat treatments and capsule hot isostatic pressings, but with little success.

Some work has been carried out on the use of acetylene in the high velocity oxyfuel thermal spraying of chromium oxide. However, acetylene is a fuel gas well-known for its tendency to decompose with violence and has to be used at relatively low pressures.

Other pressurised gas fuels have been used in high velocity oxyfuel thermal spraying processes including a stabilised mixture of methylacetylene and propadiene (MAPP). MAPP is a registered trade mark of the Air Reduction Company, Inc. MAPP is a mixture of methylacetylene and propadiene together with diluents or stabilisers such as propane and propylene. Other diluents can be present for example, methane, butane or ethane but in small percentage amounts. MAPP is used extensively particularly in the United States as a safer and more economic substitute for acetylene (see, for example, EP-A-0621079). However, difficulties have been experienced since it is customary to store liquid MAPP in a pressurised cylinder and eject the liquid MAPP as a gas under vapour pressure to employ the same in high pressure, high flow rate oxyfuel thermal spraying applications. It has been found that high vapour withdrawal rates effectively results in a fractional distillation of the MAPP gas components resulting in composition changes as the cylinder content decreases. This has been found to cause fluctuations in flame temperature and a need to adjust the flow rate of oxygen to avoid excess carbon build-up or excess oxygen.

Maintaining a constant pressure and flow rate presents further problems. This is because as the level of the liquid fuel in the pressurised cylinder decreases, the temperature likewise decreases due to the latent heat of vaporization. A reduction in temperature within the pressurised cylinder results in a reduction of pressure which adversely affects both the pressure and flow rate of the vaporized fuel stream.

It is an aim of the present invention to provide an improved method of coating a substrate with a high temperature ceramic using a high velocity oxyfuel thermal spraying technique in which the fuel gas is MAPP.

According to the present invention, a method of coating a substrate with a high temperature ceramic comprises the steps of:
a) injecting an inert gas under pressure into a container containing liquid methyl acetylene/propadiene sufficient to generate a stream of liquid methyl acetylene/propadiene;
b) removing said stream of liquid methylacetylene/propadiene from the container;
c) vaporising said stream of liquid methylacetylene/propadiene;
d) delivering the vaporised methylacetylene/propadiene through a heated and/or insulated conduit to a mixing chamber of a high velocity oxygen fuel spray gun where it is mixed with oxygen under pressure;
e) introducing said mixture into a combustion chamber of the high velocity oxygen fuel spray gun together with a powdered high temperature ceramic entrained in a stream of an inert gas; and
f) spraying the heated particles of the high temperature ceramic on to the surface of a substrate.

An embodiment of the invention will now be described, by way of example, reference being made to the Figures of the accompanying diagrammatic drawings in which:
Figure 1 is a diagrammatic sketch of an apparatus for producing MAPP gas having a substantially constant pressure, flow rate and gas composition;
Figure 2 is a diagrammatic sketch of an apparatus for coating a substrate with a high temperature ceramic and incorporating the apparatus illustrated in Figure 1; and
Figure 3 is a diagrammatic sketch of a high velocity oxyfuel gun forming part of the apparatus of Figure 2.

Referring first to Figure 1 which illustrates an apparatus 2 for generating a vaporised stream of MAPP having a substantially constant pressure, flow rate and composition. The apparatus 2 includes a storage container 4 for liquid MAPP having an inlet 6 for receiving an inert gas, for example, nitrogen via a conduit 8 extending from a pressurised nitrogen gas cylinder 10. The storage container 4 contains a tube 12 which extends almost to the floor 14 of the container and which provides a pathway for the flow of liquid MAPP when pressure is applied by the incoming nitrogen. The storage container 4 includes an outlet 16 through which pressurised liquid MAPP can pass into a conduit 18 via a flexible delivery tube 20. The flow of liquid MAPP through the conduit 18 is controlled by a valve 22.

The conduit 18 is connected to a vaporiser 24 operating at a temperature sufficient to vaporise the liquid MAPP. One such example of a suitable vaporiser is a hot water/glycol vaporiser maintained at a temperature sufficient to vaporise each component of the liquid MAPP, typically between 30 and 100°C by means of a thermostatically controlled immersion heater 26.

The flow of liquid MAPP from the conduit 18 into the vaporiser 24 is controlled by a temperature sensitive shut off valve 28 which includes a thermal probe 30 which detects the temperature of the water bath within the vaporiser. The valve 28 is operated to prevent the flow of the liquid MAPP into the vaporiser 24 until the water bath has attained a minimum desired temperature sufficient for vaporisation of the liquid MAPP. The valve 28 therefore prevents flooding of the vaporiser 24 with the liquid MAPP before it has reached operating temperature and thus avoids any liquid fuel carry over into the vaporising portion of the apparatus 2.

The vaporiser 24 transforms the liquid MAPP into a heated high pressure, high flow rate vaporised fuel stream having a temperature of typically up to about 50°C. The vaporised MAPP stream exits the vaporiser 24 through a conduit 32 controlled by a valve 34. The conduit 32 may be heated and/or insulated to prevent condensation of the vaporised MAPP stream. For example, the conduit 32 may be wrapped in a heating tape for this purpose.

In use, nitrogen from the gas cylinder 10 is fed to the storage container 4 via the conduit 8. A pressure regulator 36 is provided to ensure that the nitrogen is fed into the storage container 4 at a suitable pressure, typically from about 0.91 to 1.35 MPa about (115 to 190 psig), preferably from about 0.99 to 1.24 MPa about (140 - 175 psig).

A safety valve 38 is provided in the conduit 8 to allow the release of the nitrogen through a vent 40 when the storage container 4 has been substantially relieved of the liquid MAPP.

The nitrogen enters the head space 42 of the container 4 thereby exerting a downward force against the surface 44 of the liquid MAPP. The MAPP is therefore forced upwardly through the tube 12 and out of the outlet 16 and thus eventually into the vaporiser 24.

Referring now to Figure 2, there is illustrated an apparatus 50 for coating a substrate with a high temperature ceramic such as chromium oxide. The apparatus 50 includes a high velocity oxyfuel gun 52 (see also Figure 3) having a gas mixing chamber 54, a combustion chamber 56 and a nozzle 58 extending outwardly from the combustion chamber 56. The chambers 54, 56 are divided by a partition 55 provided with holes 57.

As shown, communicating with the gas mixing chamber 54 is a first conduit 60 connected to a source of oxygen under pressure and a second conduit 62 connected to the conduit 32 extending from the vaporiser 24.

Extending through the mixing chamber 54 and communicating directly with the combustion chamber 56 is a third conduit 64. Conduit 64 extends from a chromium oxide powder reservoir 66. A pipe 68 extends from a source of argon under pressure into the upper (as shown) end of the reservoir 66.

The gun 52 is provided with channels for a coolant, for example water.

In use, MAPP vapour is supplied to the gas mixing chamber 54 from the vaporiser 24 via conduits 32, 62 at a substantially constant pressure, flow rate and gas composition. Simultaneously, a stream of oxygen is supplied via the conduit 60 into the gas mixing chamber 54. The oxygen and the MAPP vapour are mixed in the mixing chamber and exit the mixing chamber to enter the combustion chamber 56 of the gun 52 via the holes 57 where they are ignited. Simultaneously, argon under pressure passes through the pipe 68 into the reservoir 66 where it entrains chromium oxide powder and thereafter passes through the conduit 64 directly into the combustion chamber 56. Exhaust flames and heated powdered chromium oxide particles leave the combustion chamber through the nozzle 58 and are deposited on the substrate 70.

### Example

Chromium oxide coated test samples were produced using a high velocity oxyfuel gun, having a 22 millimetre combustion chamber designed for high melting point powders. High purity chromium oxide, powder size range between 5 and 22 µm was used to spray all test samples at a powder feed rate of 25 grams per minute using high purity argon carrier gas at 11.5 litres per minute. The MAPP vapour was introduced into the combustion chamber at a pressure of 85 psi (0.59 MPa) and a flowrate of 70 l/min and the oxygen was introduced into the combustion chamber at a pressure of 150 psi (1.03 MPa) and a flow rate of 233 I/min. Surface treatment of all test samples with 40 grit alumina gave a minimum sample surface roughness (rα) of 7 - 10 µm. All test pieces were coated to a thickness between 200 - 260 µm, keeping coating temperatures below 150°C. Thicknesses greater than 380 µm were achievable.

It has been found that the deposition on a substrate of a high temperature ceramic such as chromium oxide or zirconium oxide using high velocity oxyfuel thermal spraying where the fuel gas is MAPP gas delivered at a substantially constant pressure, flow rate and composition results in a coating of high quality having very little porosity and high hardness.

## Claims

1. A method of coating a substrate with a high temperature ceramic comprising the steps of
a) injecting an inert gas under pressure into a container containing liquid methyl acetylene/propadiene sufficient to generate a stream of liquid methyl acetylene/propadiene;
b) removing said stream of liquid methyl acetylene/propadiene from the container;
c) vaporising said stream of liquid methyl acetylene/propadiene;
d) delivering the vaporised methyl acetylene/propadiene through a heated and/or insulated conduit to a mixing chamber of a high velocity oxygen fuel spray gun where it is mixed with oxygen under pressure;
e) introducing said mixture into a combustion chamber of the high velocity oxygen fuel spray gun together with a powdered high temperature ceramic entrained in a stream of an inert gas; and
f) spraying the heated particles of the high temperature ceramic on to the surface of a substrate.

2. A method as claimed in Claim 1, in which the high temperature ceramic is chromium oxide which is applied to the substrate up to a thickness of 380 µm.

3. A method as claimed in Claim 1, in which the high temperature ceramic is zirconium oxide.

4. A method as claimed in Claims 1, 2 or 3 in which the injected inert gas is nitrogen.

5. A method as claimed in any one of Claims 1 to 4 in which the high temperature ceramic is entrained in a stream of argon.

6. A method as claimed in any one of Claims 1 to 5 in which the vaporised methyl acetylene/propadiene is supplied to the mixing chamber at a substantially constant pressure, flow rate and composition.

## Patentansprüche

1. Verfahren zum Beschichten eines Substrats mit einer Hochtemperaturkeramik, mit folgenden Schritten:
a) Einblasen eines Inertgases in einen Behälter, der flüssiges Methylacetylen/Propadien enthält, unter ausreichendem Druck, um eine Strömung des flüssigen Methylacetylen/Propadiens zu erzeugen,
b) Abführen der Strömung des flüssigen Methylacetylens/Propadiens aus dem Behälter,
c) Verdampfen der Strömung des flüssigen Methylacetylens/Propadiens,
d) Befördern des verdampften Methylacetylens/Propadiens durch eine beheizte und/oder isolierte Leitung in eine Mischkammer einer Hochgeschwindigkeits-Sauerstoff-Brennstoff-Spritzpistole, wo es mit Sauerstoff unter Druck vermischt wird,
e) Einleiten des Gemischs in eine Brennkammer der Hochgeschwindigkeits-Sauerstoff-Brennstoff-Spritzpistole zusammen mit einem pulverisierten Hochtemperaturkeramikmaterial, das in einen Inertgasstrom hineingezogen wird, und
f) Sprühen der erhitzten Teilchen des Hochtemperaturkeramikmaterials auf die Substratoberfläche.

2. Verfahren nach Anspruch 1, wobei das Hochtemperaturkeramikmaterial Chromoxid ist, das mit einer Dicke von 380 µm auf das Substrat aufgebracht wird.

3. Verfahren nach Anspruch 1, wobei das Hochtemperaturkeramikmaterial Zirkoniumoxid ist.

4. Verfahren nach Anspruch 1, 2 oder 3, wobei das eingeblasene Inertgas Stickstoff ist.

5. Verfahren nach einem der Ansprüche 1 bis 4, wobei das Hochtemperaturkeramikmaterial in einem Argonstrom mitgeführt wird.

6. Verfahren nach einem der Ansprüche 1 bis 5, wobei das verdampfte Methylacetylen/Propadien der Mischkammer mit im wesentlichen konstantem Druck, konstantem Strömungsdurchsatz und konstanter Zusammensetzung zugeführt wird.

## Revendications

1. Procédé de revêtement d'un substrat avec une céramique pour hautes températures, comprenant les étapes de :
(a) injection, dans une cuve contenant un mélange liquide méthyl-acètylène/propadiène, d'un gaz inerte sous pression suffisante pour générer un courant du mélange liquide méthyl-acétylène/ propadiène ;
(b) retrait dudit courant du mélange liquide méthyl-acétylène/propadiène de la cuve ;
(c) vaporisation dudit courant du mélange liquide méthyl-acétylène/propadiène ;
(d) fourniture du mélange méthyl-acètylène/propadiène vaporisé via une canalisation chauffée et/ou isolée à une chambre de mélange d'un pistolet de pulvérisation à haute vitesse par flamme d'oxygène et de combustible (HVOF) où il est mélangé avec de l'oxygène sous pression ;
(e) introduction dudit mélange dans une chambre de combustion dudit pistolet de pulvérisation à haute vitesse par flamme d'oxygène et de combustible (HVOF) simultanément avec une céramique en poudre pour hautes températures entraînée dans un courant d'un gaz inerte ; et
(f) pulvérisation des particules chauffées de céramique pour hautes températures sur la surface d'un substrat.

2. Procédé selon la Revendication 1, dans lequel la céramique pour hautes températures est l'oxyde de chrome qui est appliqué sur le substrat sur un épaisseur allant jusqu'à 380 µm.

3. Procédé selon la Revendication 1, dans lequel la céramique pour hautes températures est l'oxyde de zirconium.

4. Procédé selon les Revendications 1, 2 ou 3, dans lequel le gaz inerte injecté est l'azote.

5. Procédé selon l'une quelconque des Revendications 1 à 4, dans lequel la céramique pour hautes températures est entraînée dans un flux d'argon.

6. Procédé selon l'une quelconque des Revendications 1 à 5, dans lequel le mélange méthylacétylène/propadiène vaporisé est fourni à la chambre de mélange sous une pression, un débit et une composition sensiblement constants.
